

## UNITED STATES PATENT OFFICE

2,520,081

METACHROME DYEING PROCEDURE AND  
PRODUCTS DYED THEREWITH

Chester A. Amick, Bound Brook, and George L. Royer, North Plainfield, N. J., assignors to American Cyanamid Company, New York, N. Y., a corporation of Maine

No Drawing. Application December 7, 1948,  
Serial No. 64,037

6 Claims. (Cl. 8—30)

1

This invention relates to an improved metachrome process in which basic nitrogenous fibres such as wool are dyed in a metachrome bath containing a suitable salt or compound of chromium for metallizing purposes and a soluble salt of a metal of the B family of the second group of the periodic system.

The ordinary metachrome process is used to dye wool and similar fibres by means of a dye bath which contains a soluble chromium compound, the dyeing usually proceeding on the acid side. The metachrome process has been used practically only with a few colors because with many colors it has been difficult to obtain a dyeing of suitable strength and levelness. It has been proposed in the past to increase the penetration by the presence of a cationic surface active agent but this has not proven satisfactory in practical operation because the cationic surface active agent reacts with the constituents of the dye bath to produce insoluble colored material which tends to form a colored scum resulting in spotty or uneven dyeing.

In the prior patent of which we are inventors No. 2,434,178 there is described a metachrome process in which the difficulties of scum formation have been avoided by using a colloidized cationic surface active agent. This resulted in a great advance and made the metachrome process practical in many instances where it was formerly not considered suitable. However, the maximum strength obtainable was not greatly increased over that which was known before and this still left room for an improved process which could retain the level dyeing but produce a still stronger shade.

The present invention achieved such a result by the addition of two features to the dyeing process claimed in the earlier patent. The first and most important feature is the presence of a soluble compound of a metal of the B family of the second group of the periodic system. This family includes the well known metals zinc and cadmium. The second feature is that the pH of a dye bath to start is alkaline but not greater than 9.5 and is gradually rendered more acid until finally the acidity reaches a point not lower than the isoelectric point of wool, about pH 4.0 at the end of the dyeing procedure.

The mechanism by which the salts of the metals of the B family of the second group of the periodic system act to produce increased strength of shade is not known. It does not appear to be a question of the metals actually adding on to

2

the complex because there are sufficient chromium compounds present to completely metallize the dye before the dyeing is completed. It is therefore not desired to limit the present invention to any particular theory of why the increased strength of shade is obtained.

Except for the change in pH during the dyeing procedure no new techniques need to be learned by the dyer as the process proceeds in a manner which is conventional in the dyeing of wool by the metachrome process. This is a practical advantage. The addition of acid is not a critical matter, any suitable acid which does not react with the dyestuffs may be employed. For this purpose acetic acid presents many practical advantages and is the preferred acid although the ordinary mineral acids such as hydrochloric and sulfuric acids may also be used.

It is an advantage of the present invention that strong dyeings are obtainable with all of the ordinary chrome dyes which are susceptible to the metachrome process and even some which were not considered suitable in the past. In fact the general applicability of the process to chrome colors is one of its most important practical advantages. While the process may be used with a wide number of dyestuffs nevertheless it should be realized that there is some variation in behavior from dyestuff to dyestuff and therefore the invention is of particular importance in connection with those dyes which are readily dyed by the metachrome process where shades and maximum strength are desired. On the other hand when such great strength is not required the present invention opens up the field of metachrome dyeing to a number of dyes which were not of practical importance hitherto.

Although the improved strength of shade, levelness of dyeing and good penetration is perhaps the most important single result of the present invention it is a further advantage that exhaustion is more complete which results in a saving in the amount of dye used. Where the cost of the dyestuff is an important factor this represents a real practical economy.

The invention will be described in greater detail in conjunction with the specific examples which are typical embodiments. The parts are by weight.

50

## Example 1

A dye bath is prepared as follows: 10 parts of a dyestuff having Color Index No. 203, predissolved in boiling water, 10 parts of 28% aqueous ammonium hydroxide, 5 parts of a nonionic sur-

face active agent prepared by reacting 2 mols of polyethylene oxide (molecular weight 4,000) and 1 mol of the dimerized acid obtained by heat treating soya bean acid and distilling off the monomeric acid, 2½ parts of the condensation product of octadecylguanidine bicarbonate and 6 parts of ethylene oxide, 10 parts of cadmium chloride, 3 parts of potassium bichromate, and water to bring the volume of the bath up to 40,000 parts.

500 parts of woolen yarn or goods are prewet with water and entered into the dye bath at 110° F. The dye liquor is brought to the boil in half an hour with frequent turning of the wool to insure uniform dyeing. Boiling and turning are continued for another half hour after which 10 parts of 28% acetic acid are added and boiling and turning continued for a further half hour. Then 20 parts of 28% acetic acid is added and boiling and turning continued for a third half hour.

A control dyeing is made by the usual metachrome process, the bath consisting of 10 parts of dyestuff previously dissolved in boiling water, 50 parts of ammonium sulfate, 5 parts of potassium bichromate and sufficient water to bring up the dye bath to 40,000 parts.

The wool dyed by the first bath when examined by a recording spectrophotometer shows an increase in strength over the control dyeing of about 232%.

#### Example 2

The procedure of Example 1 is repeated but 10 parts of zinc chloride are used in place of the cadmium chloride. A skein dyed in the presence of the zinc chloride is about 265% stronger than the control dyeing.

#### Example 3

The procedure of Example 2 is repeated but using a different dyestuff having Color Index 652. The strength of the dyed wool is 95% greater than the control dyeing.

#### Example 4

The procedure of Example 1 is followed using the dyestuff of Example 3. The wool dyed in the bath containing the cadmium salt has a strength 75% greater than that of the control dyeing.

#### Example 5

The procedure of Example 1 is followed but a different dyestuff is used having Color Index No. 1034. The wool dyed in the bath containing cadmium chloride is 28% greater in strength than the control value.

#### Example 6

The procedure of Example 1 is followed using, however, a dyestuff having a Color Index No. 299. The color value of the dyed goods from the bath containing the cadmium chloride is 40% greater than that of the control dyeing.

#### Example 7

The procedure of Example 1 is repeated ex-

cept the dyeing is made on nylon. The dyeing made in the bath containing the preferred features is very much stronger than that made in the control bath.

6

#### Example 8

Procedure of the preceding example is repeated exactly except the dyeing is made on real silk. Again the color value of the dyeing and the penetration of the fibers is excellent.

We claim:

1. A method of dyeing which comprises subjecting a substantially unmetallized basic nitrogenous fiber to the action of a dye bath formed by mixing a chromable dye, a soluble chromium compound, a cationic surface active agent, a soluble salt of a metal of group II—b of the periodic system, water, and sufficient alkali to make the pH of the bath alkaline but not greater than 9.5 and to cause said dye to react with said group II—b metal salt to form a group II—b metal complex of said dye, partially dyeing said fiber from said complex, gradually lowering the pH of said bath to a point where decomposition of said complex and chromation of the dye take place, and completing the dyeing at a pH of not less than about 4.0.

2. A method according to claim 1 in which the basic nitrogenous fibre is wool.

3. The method according to claim 2 in which the soluble compound of the metal of the B family of the second group of the periodic system is a soluble cadmium salt.

4. A method according to claim 3 in which a cationic surface active agent is a condensation product of octadecylguanidine bicarbonate and ethylene oxide.

5. A method according to claim 2 in which the metal of the B family of the second group of the periodic system is zinc.

6. A method according to claim 5 in which the cationic surface active agent is a condensation product of octadecylguanidine bicarbonate and ethylene oxide.

45 CHESTER A. AMICK.  
GEORGE L. ROYER.

#### REFERENCES CITED

The following references are of record in the file of this patent:

#### UNITED STATES PATENTS

| Number     | Name      | Date          |
|------------|-----------|---------------|
| 661,985    | Haussmann | Nov. 20, 1900 |
| 55 941,399 | Winslow   | Nov. 30, 1909 |
| 2,434,178  | Royer     | Jan. 6, 1948  |

#### FOREIGN PATENTS

| Number     | Country | Date          |
|------------|---------|---------------|
| 60 821,992 | France  | Sept. 6, 1937 |

#### OTHER REFERENCES

Amer. Dyes. Rep. for Sept. 8, 1947, page P495.  
"Smith's Inorganic Chemistry," revised by  
65 Kendall, published in N. Y. C. by Century Co.,  
1926, page 794.